

## UNITED STATES PATENT OFFICE

2,198,719

## PROCESS OF HARDENING COPPER ALLOYS

Claude H. Coleman, Fairmead, Calif.

No Drawing. Application November 20, 1937,  
Serial No. 175,673

2 Claims. (Cl. 148—13.2)

The invention generally relates to the treatment of copper for hardening the same and more particularly relates to a tempering process which is carried out without the alloying of any element with the commercially pure copper or copper alloy subjected to the process.

The present application is a continuation in part of my co-pending application entitled "Process of tempering copper", filed December 31, 1935, and bearing Serial No. 57,065.

I have carried out my process in connection with commercially pure copper and copper alloys fabricated in a form suitable for use as bearings and have found, as indicated by the following examples, that the process hardens the metal to an extent that the wearing properties of the bearings made from such metals have been appreciably enhanced. I have also found that commercially pure copper and copper alloys treated in accordance with the process of my invention lends itself more readily to polishing and the retention of polished surfaces for a greater period of time. Moreover, I have treated commercially pure copper stock that has been cast in the form of bells, and have found that the tonal qualities of the treated bells are far superior to cast copper bells that are not treated in accordance with my process.

It is perhaps well known that there has been heretofore but two recognized methods of hardening copper. One method, apparently practiced by primitive peoples, comprises the mechanical treatment of the copper such as by hammering to effect hardened cutting edges on copper fabricated tools. The other method comprises heat treatment of copper charges, as by melting the same. As to this latter method, the authorities are in accord with the view that during such heat treatment the metal becomes thoroughly impregnated with cuprous oxide so that in effect the metal is alloyed with the oxide. Consequently, it is said that copper can be hardened either by mechanically working the same or by alloying some other element with it. My process, as hereinafter described, does not involve the mechanical working of the metal nor does it entail the alloying therewith of any other element. Moreover, the process is equally applicable to the hardening of copper alloys as well as to the hardening of substantially pure copper.

It is an important object of my invention to provide a process of treating either commercially pure copper or copper alloys to afford an increased hardness throughout the treated metal or alloy and enable the efficacious use of the

treated metal or alloy as tools or bearings or desired polished copper products, including copper bells.

A further object of the invention is to provide an improved and inexpensive process for materially hardening a substantially pure copper, such as commercially pure copper, or a copper alloy such as bronze or brass, without alloying any element therewith.

A still further object of the invention is to provide improved metals and metal alloys that are readily polished and that maintain a polished surface for appreciable periods of time.

Another object of the invention is to provide a process of tempering commercially pure copper or copper alloys without subjecting the same to reaction with oxides.

Other objects of the invention, together with some of the advantageous features thereof, will appear from the following description of a preferred mode of carrying out the process. It is to be understood that I am not to be limited to the precise method set forth nor to the precise solutions employed in the process as the invention, as defined in the appended claims, may be carried out in a plurality and variety of ways with a plurality and variety of solutions.

The invention contemplates the use of beef tallow as one solution in which the copper is immersed or as an equivalent thereof either a petroleum or a vegetable oil. I have found that cottonseed oil can be employed with effective results. Moreover, the process involves the use of a soap solution maintained at boiling temperature. A preferable soap solution is either sodium stearate or sodium palmitate and it is preferred that the solution have a density of approximately 1.009. Another soap that I have used with efficacious results contained approximately 6.25% of moisture, 23.85% of alkali in the form of sodium carbonate, approximately 70.60% of fatty matter which consisted of cottonseed stearine, and free caustic alkali which was sodium hydroxide. This soap has a specific gravity at 100° C. of 0.867 and solidifies at 30° C.

In accordance with the invention, the commercially pure copper or alloy thereof to be tempered is initially chilled. Preferably the temperature of such metal or alloy is reduced to ten degrees (10°) below zero degrees (0°) Fahrenheit or lower. I have found that the commercially pure copper or alloy thereof to be hardened can be initially chilled to a temperature approximately as low as 120° below 0° Fahrenheit and its

hardness materially increased by following the hereinafter set forth cycle of steps.

After the commercially pure copper or alloy thereof has been chilled to 10° below 0° Fahrenheit or lower, it is immersed for a period of twenty (20) seconds, more or less, depending upon the thickness of the piece of stock used, in a hot bath of either beef tallow, a vegetable oil or a petroleum oil and then transferred from that bath to a boiling soap solution. Preferably, the initial temperature of the bath of beef tallow, or vegetable oil or petroleum, is fixed at approximately 240° Fahrenheit and, since the preferable soap solution is either sodium palmitate or sodium stearate, it is clear that the temperature of the boiling soap solution is approximately 205° Fahrenheit. In passing the stock from the beef tallow or oil bath to the soap solution, the material is not wiped but is permitted to retain the envelope of film of tallow or oil which it picks up upon immersion therein. Thus it is not exposed to the air.

The period of time for immersion of the commercially pure copper or alloy thereof in the solution preferably is approximately thirty (30) seconds, more or less, depending, of course, upon the thickness of the piece of stock being treated. After such period has elapsed the stock is withdrawn from the soap solution and thoroughly wiped and dried to free it entirely of the soap solution as well as any film of oil or beef tallow that may have been retained thereon. The stock is allowed to cool to room temperature and then the foregoing cycle is repeated with the exception that the temperature of the bath of beef tallow is first raised to approximately 280° F. After the second cycle has been completed, and for every cycle of operations thereafter, the temperature of the beef tallow bath is raised in steps of 10° until a temperature of approximately 400° Fahrenheit is reached, at which temperature the beef tallow bath is maintained during further cyclic steps.

If desired, a hardness test may be made after each cycle of operations to ascertain the percentage of increase or actual increase in hardness of the material. If a definite or certain hardness is desired, the foregoing cycle is to be repeated until such hardness is attained unless it be found that after a certain number of cycles an apparent hardness has been reached which will be maintained even though repeated cyclic operations are carried out.

It is to be noted that in addition to cleansing the commercially pure copper or alloy thereof, the immersion in the soap solution effects a gradual reduction of the temperature while at the same time keeping the material out of contact with the air, thus avoiding formation of oxides and the impregnation of the material with oxides.

While I have mentioned above that mineral or vegetable oils may be substituted for the beef tallow solution, I prefer to employ the beef tallow since it will retain a higher temperature than such oils and will heat the above mentioned metal more evenly leaving it tougher and with a finer grain.

The following examples are indicative of the increased hardness effected in certain commercially pure copper stock and copper alloys tempered in accordance with my foregoing process:

#### EXAMPLE I

75 An annealed copper rod, purchased in the open

market, was cut into bars and numbered 1 to 8 inclusive for identification. A spectrograph analysis of this rod before treatment was made and indicated the presence of the following elements in the percentages indicated:

|                         | Per cent   |
|-------------------------|------------|
| Zinc—approximately      | 0.001      |
| Silicon—approximately   | 0.001      |
| Silver—approximately    | 0.001      |
| Lead—approximately      | 0.0001     |
| Chromium—approximately  | 0.0001     |
| Magnesium—approximately | 0.0001     |
| Copper (by difference)  | 99.99 plus |

Each of the blocks numbered 1 to 8 inclusive were tested for hardness before treatment with my aforementioned and described process. The hardness value of each block, measured on the Rockwell F scale, and resulting from three readings in each case, was as follows:

| #1   | #2   | #3   | #4   | #5   | #6   | #7   | #8   |
|------|------|------|------|------|------|------|------|
| 25.0 | 28.7 | 28.3 | 27.0 | 31.7 | 32.0 | 31.3 | 31.3 |

Two of these blocks—namely, numbers 5 and 7, were then subjected to the process of my invention and hardness readings were taken at the end of approximately 80 cycles. The following hardness values, taken at the end of 80 cycles through my process, are the result of averages of three readings in each instance:

|      |      |
|------|------|
| #5   | #7   |
| 40.7 | 43.7 |

A spectrograph analysis of blocks #5 and #7 was then made and indicated the same elements to be present in the same percentages as before, or, in other words, that no alloying had taken place as a result of the treatment. The spectrograph analysis of blocks #5 and #7 were the same and showed the following:

|                         | Per cent   |
|-------------------------|------------|
| Zinc—approximately      | 0.001      |
| Silicon—approximately   | 0.001      |
| Silver—approximately    | 0.001      |
| Lead—approximately      | 0.0001     |
| Chromium—approximately  | 0.0001     |
| Magnesium—approximately | 0.0001     |
| Copper (by difference)  | 99.99 plus |

#### EXAMPLE II

The same procedure was carried out with respect to specimens from a 1/4" square hard drawn copper rod purchased in the open market. Four blocks numbered 9 to 12 for identification, were cut from the bar. A spectrograph analysis of the bar was made both before and after treatment and hardness values were obtained by striking an average from three readings. These hardness values were ascertained both before treatment as well as after treatment in accordance with my herein above described process. The spectrograph analysis of the hard drawn copper bar before treatment showed the presence of the following elements in the percentages indicated:

|                        | Per cent   |
|------------------------|------------|
| Silver—approximately   | 0.0001     |
| Calcium—approximately  | 0.00001    |
| Copper (by difference) | 99.99 plus |

The hardness values of blocks numbered 9 to 12 inclusive cut from such hard drawn copper rod

were as follows, these values being the average of three readings on the Rockwell F scale and represent the hardness values before treatment:

| #9   | #10  | #11  | #12  |
|------|------|------|------|
| 75.3 | 81.7 | 82.0 | 82.0 |

The blocks numbered 10 and 11 were subjected to the treatment as above described and Rockwell hardness values on the F scale were ascertained by striking an average of three readings in each instance. The cycle of operations was carried out in each instance approximately 80 times. The hardness values of blocks #10 and #11 after treatment were as follows:

| #10  | #11  |
|------|------|
| 84.7 | 85.0 |

A spectrograph analysis of both blocks #10 and #11 was then made after treatment as aforesaid and the spectrograph analysis indicated that the blocks were the same as before or, in other words, no alloying had taken place. The analysis of blocks #10 and #11 after treatment is as follows:

|                        | Per cent   |
|------------------------|------------|
| Silver—approximately   | 0.0001     |
| Calcium—approximately  | 0.00001    |
| Copper (by difference) | 99.99 plus |

#### EXAMPLE III

A 1 5/8" round cast copper rod, purchased in the open market, was cut into five blocks and numbered 1 to 5 inclusive. Hardness values before and after treatment were measured and spectrograph analysis made both before and after treatment. The spectrograph analysis of the cast copper rod before treatment indicated the presence of the following elements, in the percentages indicated:

|                         | Per cent  |
|-------------------------|-----------|
| Tin—approximately       | 0.4       |
| Silicon—approximately   | 0.001     |
| Silver—approximately    | 0.05      |
| Lead—approximately      | 0.001     |
| Chromium—approximately  | 0.0001    |
| Magnesium—approximately | 0.0001    |
| Copper (by difference)  | 99.5 plus |

The hardness value of each of the blocks numbered 1 to 5 inclusive, which were cut from the round cast copper rod, was, before treatment, 26 on the Rockwell F scale, such value being the average of three readings.

After treating block number 4 and carrying the block through approximately 80 cycles, the Rockwell F scale hardness value thereof obtained by taking an average of three readings was 50.0.

The spectrograph analysis of block #4 from the round cast copper rod showed, after treatment, the presence of the following elements in the percentages indicated:

|                         | Per cent  |
|-------------------------|-----------|
| Tin—approximately       | 0.4       |
| Silicon—approximately   | 0.001     |
| Silver—approximately    | 0.05      |
| Lead—approximately      | 0.001     |
| Chromium—approximately  | 0.0001    |
| Magnesium—approximately | 0.0001    |
| Copper (by difference)  | 99.5 plus |

thus indicating that no alloying had taken place.

#### EXAMPLE IV

In addition to the foregoing tests, specimens of substantially pure copper as well as specimens of brass were treated in accordance with my process and tests were made not only for hardness values but also for characteristics indicating the value of the treated metal and metal alloy as applied to bearings. The specimens were subjected to spectrograph analysis before and after treatment and also were tested for hardness throughout their cross-sectional areas. The particular specimens so treated were marked for indication. One specimen consisting of a block of cold rolled copper, marked #2 for identification, was examined before treatment and the spectrograph analysis showed its composition to be as follows:

|                         | Per cent      |
|-------------------------|---------------|
| Lead—approximately      | 0.001         |
| Silver—approximately    | 0.003         |
| Calcium—approximately   | 0.001         |
| Aluminum—approximately  | 0.0001        |
| Silicon—approximately   | 0.0001        |
| Magnesium—approximately | 0.0001        |
| Copper (by difference)  | 99.99 plus 25 |

The hardness value of copper block #2, measured on the Rockwell F scale was 47, such value being the average of three (3) readings of the scale. The block was then subjected to the process of my invention and the spectrograph analysis showed its composition to be, after treatment, as follows:

|                         | Per cent      |
|-------------------------|---------------|
| Lead—approximately      | 0.001         |
| Silver—approximately    | 0.003         |
| Calcium—approximately   | 0.001         |
| Aluminum—approximately  | 0.0001        |
| Silicon—approximately   | 0.0001        |
| Magnesium—approximately | 0.0001        |
| Copper (by difference)  | 99.99 plus 40 |

thus showing that no alloying had taken place in the treatment.

The treated copper block marked #2 for identification was then tested not only for surface hardness but for hardness throughout its cross-section. The surface hardness value, on the Rockwell F scale, was 75 which value is an average of three (3) readings on the scale. The block was then cut into two pieces and tested for hardness on the cut surface. The hardness value on the cut surface of the treated block was found to be 76.3, an average of three readings on the Rockwell F scale. As a result of the treatment of block #2, in accordance with my process, the hardness value was raised from 47 to 75 on the outside surface and to 76.3 on the inside, a result of three readings on the Rockwell F scale.

#### EXAMPLE V

A friction and wear test on a Timken machine was made with respect to a medium hard, cold rolled copper block, marked #1 for identification, this being from stock purchased in the open market. The test was made on this stock prior to treatment and then subsequent to the cyclic treatment in accordance with my process. During the duration of the test, which was for two hours, a load of 3,900 pounds per square inch was put on the copper block and a speed of 400 revolutions per minute was maintained. The oil temperature, using an oil having an S. A. E. rating of 30, was 130° F. during the period of the test.

The copper block, marked #1 for identification, was then weighed and the loss due to wear and the coefficient of friction were calculated. Sum-

marizing this test, the results may be set forth as follows:

5 *Timken friction and wear test on copper block marked #1 for identification—after treatment*

Original weight of block  
(untreated) 25.9932 grams  
Final weight (treated) 25.9820 grams  
10 Loss due to wear 0.0112 gram  
Coefficient of friction 0.014 gram  
Duration of test 2 hours  
Oil used Golden Shell SAE 30  
15 Temperature of oil 130° F.  
Speed 400 R. P. M.  
Initial load on bearing 3,900 lbs. per sq. inch

EXAMPLE VI

20 The process of my invention was also carried out with respect to a copper alloy purchased from stock in the open market. Specifically, a brass block was obtained and cut into two pieces. One piece was marked with the letter "V" for identification, while the other piece was unmarked. The unmarked piece was not treated. Spectrograph analysis were made of the untreated and treated blocks and indicated the following composition:

| 30 |                         | 1/2 brass block (untreated) | 1/2 brass block (treated) |
|----|-------------------------|-----------------------------|---------------------------|
| 35 | Copper—approximately    | Percent<br>65.0             | Percent<br>65.0           |
|    | Zinc—approximately      | 33.0                        | 33.0                      |
|    | Lead—approximately      | 2.0                         | 2.0                       |
|    | Tin—approximately       | 0.001                       | 0.001                     |
|    | Silver—approximately    | 0.001                       | 0.001                     |
|    | Calcium—approximately   | 0.001                       | 0.001                     |
|    | Aluminum—approximately  | 0.0001                      | 0.0001                    |
|    | Silicon—approximately   | 0.0001                      | 0.0001                    |
| 40 | Magnesium—approximately | 0.0001                      | 0.0001                    |

These analysis established that no alloying resulted from the treatment of the brass block in accordance with my process.

45 The two pieces of brass, as aforesaid, were then tested for hardness on the Rockwell F scale. The surface hardness value of the brass block before treatment was found to be 85, this value being the average of three readings of the scale. The surface hardness value of the brass block after treatment was found to be 90, this value being the average of three readings on the scale. The treated brass block, marked "V" for identification, was then cut into two pieces and the cut surface was tested for hardness to indicate whether or not the treatment had effected an increased hardness throughout the cross-section of the block. The hardness value of the cut surface, measured on the Rockwell F scale, was found to be 91, this value being an average 50 of three readings of the scale.

In addition to the foregoing tests, abrasion or friction and wear tests were made in connection with the brass blocks, treated and untreated, on a Timken machine. The results of these tests 65 are as follows:

Timken friction and wear tests

| 70               |       | Unmarked and untreated brass block | Treated brass block, marked "V" |
|------------------|-------|------------------------------------|---------------------------------|
| Initial weight   | grams | 53.2258                            | 54.1714                         |
| Final weight     | do    | 52.2828                            | 53.4980                         |
| Loss due to wear |       | 00.9430                            | 0.7134                          |

75 thus establishing that the wear on the untreated

brass block was 32.18% greater than the wear on the brass block treated in accordance with my process.

The mechanical and temperature conditions of these friction and wear tests on the brass blocks were as follows:

Duration of tests—each  
test 2 hours  
Speed—each test 400 R. P. M.  
Oil used—each test Golden Shell SAE 30  
Temperature of oil—each  
test 130° F.  
Initial load—each test 3920 lbs. per sq. inch  
Final load—each test 274 lbs. per sq. inch  
Average load—each test 2097 lbs. per sq. inch

EXAMPLE VII

A specimen of the cast copper rod referred to in Example III was also subjected to a friction and wear test. Three pieces of the specimen were marked #2, #4 and #5 for identification. The piece marked #2 was put through approximately 40, more or less, cycles of my process while the piece marked #4 was put through approximately 80, more or less, cycles of the process. The piece marked #5 was untreated. As indicated in Example III, the hardness value of the untreated specimen was 26. After treatment, as aforesaid, the piece marked #2 had a hardness value of 39 measured on the Rockwell F scale, such value being the average of three readings. After treatment, the piece marked #4 had a hardness value of 50 measured on the Rockwell F scale, such value being the average of three readings. The friction and wear tests on these three specimens resulted as follows:

Timken friction and wear tests

|               | Block No. | Coefficient of friction | Loss in weight | 4      |
|---------------|-----------|-------------------------|----------------|--------|
| 2             |           |                         | Grams          |        |
| 4             |           |                         | 0.100          | 0.0056 |
| 5 (untreated) |           |                         | 0.054          | 0.0014 |
|               |           |                         | 0.156          | 0.0075 |

thus showing that the untreated copper piece (#5) lost five and one-third times as much weight as the fully treated block or piece #4 while the piece treated only one-half as much as the latter, that is block #2, lost four times as much weight as the fully treated piece #4. Consequently, these tests established that copper treated in accordance with my process withstands wear to a much greater extent than untreated copper.

EXAMPLE VIII

A test was next made to compare the wearing qualities of an untreated block of Tobin bronze with a piece of commercially pure copper treated in accordance with my process. The copper block was run through approximately 80 cycles of the process. The block of Tobin bronze was marked #1 for identification and the block of copper, so-treated, was marked #2 for identification. The results of the friction and wear tests is as follows:

Timken friction and wear tests

|                           | #1 untreated Tobin bronze | #2 treated copper block | 70 |
|---------------------------|---------------------------|-------------------------|----|
| Original weight of blocks | Grams                     | Grams                   |    |
| Final weight              | 25.1062                   | 27.3916                 |    |
| Loss due to friction      | 23.6251                   | 27.2553                 |    |
| Coeff. of friction        | 1.4811                    | 0.1363                  |    |
|                           | .02                       | .11                     |    |

thus showing that the Tobin bronze block not treated by my process lost eleven times as much weight during the test than the copper block treated in accordance with my process. The conditions of test were identical for each block and were as follows:

Initial load on bearing 3900 lbs per sq. inch  
 Speed 400 R. P. M.  
 Oil used Golden Shell, S. A. E. 30  
 Temperature of oil 139° F.  
 Duration of test Two hours

The foregoing examples of tests of copper and copper alloys treated in accordance with the herein described process establish that not only does the process effect an increase in the surface hardness of the copper and copper alloys but also an increased hardness throughout the cross-sectional dimensions of the material. The process, therefore, possesses commercial utility in that bearings made from commercially pure copper or alloys thereof treated in accordance with the process have a definitely increased resistance to wear and an increased resistance to loss in weight due to friction.

By subjecting such metals as commercially pure copper and alloys thereof to the process hereinabove described, I have found that the outer surfaces of the copper and copper alloys have been rendered appreciably resistant to oxidation and further that such surfaces are readily polished and will retain a polished condition for relatively long periods of time.

The increased hardness of the commercially pure copper and copper alloys as effected by my process renders the resultant products capable of many industrial uses to which the specific metal could not heretofore be used. One new use of a substantially pure copper treated in accordance with my process is in the form of sheets disposed on aeroplane wings. The hardened and polished copper sheets on the wings could be readily heated and ice and snow thus kept from adhering thereto.

5 It is to be understood that whenever the terms "substantially pure copper" and "commercially

pure copper" are used in this specification, the terms shall be construed to mean copper that contains less than one per cent (1%) of impurities.

The appended claims are to be accorded a range of equivalents commensurate in scope with the advance made over the prior art.

I claim:

1. A process of treating copper alloys to increase the hardness thereof, said process comprising the steps of reducing the temperature of the metal from normal room temperature to at least the freezing temperature of water, then immersing the chilled metal in a tallow bath having a temperature of at least 240° F. and maintaining the metal therein for at least 20 seconds, then transferring the metal from the tallow bath to a boiling soap solution and maintaining the same therein for at least 20 seconds, removing the metal from said soap solution, drying the same and allowing the metal to return to normal room temperature, and repeating the aforesaid steps as required to obtain the desired degree of hardness of the metal, the reduction of temperature of said metal on the second and subsequent repetitions being to approximately -10° F.

2. The improved process of hardening an alloy consisting of approximately 65% copper, 33% zinc and 2% lead, said process comprising the steps of first reducing the temperature of said alloy from normal room temperature to at least the freezing temperature of water, then immersing said alloy in a tallow bath having a temperature of at least 240° F. and maintaining said alloy in said bath of tallow for at least 20 seconds, transferring said alloy from said tallow bath to a boiling soap solution and maintaining the same in said soap solution for at least 20 seconds, removing said alloy from said soap solution, drying the same and allowing it to return to normal room temperature, and then repeating the aforesaid steps as required to attain the desired degree of hardness, the reduction of temperature of said alloy on the second and subsequent repetitions being to approximately -10° F.

CLAUDE H. COLEMAN.